

**1****3,699,028**

**NON-WOVEN FABRICS BY ELECTRODEPOSITION**  
Robert Edward Torley, Wilton, and Richard Dale Bankert,  
Norwalk, Conn., assignors to American Cyanamid  
Company, Stamford, Conn.  
No Drawing. Filed Oct. 1, 1971, Ser. No. 185,875  
Int. Cl. B01d 13/02; B01k 5/00; C23b 7/00  
U.S. Cl. 204—180 R **8 Claims**

**ABSTRACT OF THE DISCLOSURE**

Non-woven fabric webs of fiber and binder resin are formed at one electrode of an electrolytic cell from a dilute bath of fibers and resin in aqueous suspension. Soft, pliable webs are obtained by using very dilute suspensions having less than one percent by wt. fiber and less than 0.2 percent by wt. resin in the aqueous coating bath and having one to five parts fiber per one part resin in said bath.

The invention relates to manufacture of non-woven fabrics and articles of such fabric by electrophoretic deposition from aqueous dispersions of fiber staple or flock dispersed in aqueous bath with resin binder.

Non-woven fabrics of fiber staple and flock have been made by several methods, usually by depositing the fibers in a suitable paper making method or in a dry lay process and subsequently impregnating the deposit of fibers with resin binder.

The invention provides improvements in electrophoretic coating process whereby the electrophoretic process is adapted to the making of non-woven fabrics having properties that are comparable with and in some instance superior to those non-woven fabric products of the paper making and dry lay processes.

Electrophoretic coating methods have been used successfully for applying resin and pigment paint to metal and other conductive surfaces such as wires, plates, screens and the like. In addition to ordinary pigments, other solid materials such as carbon, graphite and asbestos fibers, mica, and the like have been included in the electrophoretically coated material with suitable resins. Not all electrophoretic processes have the purpose of painting or insulating the electrode surface. Electrophoresis has been used for forming sheets, films and the like on an electrode, from which the deposited sheet or film is then removed for use as such apart from the electrode. U.S. Pat. No. 3,449,227, patented June 10, 1969 to G. F. Heron et al. describes an electrophoretic process for making sheets, tapes, yarns and the like with asbestos fibers or other mineral fibers. The process of the present invention differs from the process described in the Heron patent essentially by substantial differences in the concentrations of the resin and the relative concentrations of resin and fiber materials in the electrolyte baths that are used in the respective processes. Because of those essential process differences, and because the present invention may use other fibers than asbestos, the non-woven fiber products are of substantially different texture and composition than the products described in the Heron patent.

The invention produces non-woven fiber sheets or articles which are essentially self-supporting fabric webs of synthetic and natural cellulosic fiber staple or flock, or the like, or mixtures of such staple and flock fibers, bound with a synthetic resin binder. This self-supporting web material in some of our most preferred embodiments has a fleecy or flocculent outer surface but in several embodiments the fabric products may be modified in texture, thickness, density, porosity and permeability to some extent by variations in the selection of materials and by variation of the process conditions and by after-treating

**2**

methods such as curing and calendering. The fabric products have sufficient dry strength to be self-supporting for many uses, but are also adaptable for fabrication with a scrim or backing material for additional strength if desired. The invention has the advantage that in some embodiments shaped articles of fabric can be formed directly to a desired shape by electrodeposition of the fabric on a suitably shaped electrode mold. Fabric sheets, tubes, tapes, cups, preformed articles of clothing, and other shaped fabric articles such as irregular shaped toys, mitts and the like can be formed directly by deposition of the fiber and binder on shaped electrode surfaces and removing the formed articles from the electrode. The web fabric attains structural integrity and some wet strength as it is formed on the electrode due to the presence of resin binder in the web fabric. The process is especially advantageous for making disposable non-woven fabric articles such as disposable towels, napkins, sheets, clothes and the like.

20 In a process according to the invention, an aqueous suspension is prepared comprising dispersed synthetic fiber staple or flock or a mixture thereof suspended in the bath and synthetic resin binder which is either coated on the fiber surfaces in some embodiments, or more often 25 is present suspended as finely divided resin particles dispersed in the aqueous electrolyte bath. The suspension usually will also comprise a soluble emulsifying agent to maintain the fiber and binder in the dispersion. However, in a few instances the binder resin may possess inherent 30 surface active properties adequate for this dispersing function. Immersed in the aqueous bath is a working electrode on which the fiber and resin are to be electrophoretically deposited. Usually but not in all instances the working electrode is the anode. A counter electrode of opposite 35 polarity will also contact the aqueous suspension, separated from the working electrode, to complete the cell. The electrodes are connected electrically to a direct current external power source and current is supplied at voltage sufficient to cause the fiber and resin to be co-deposited at the working electrode.

After the desired fabric of fiber and resin has been formed by electrophoretic deposition on the anode, the fabric is stripped from the electrode. In some embodiments the electrode is removed from the suspension and 45 the fabric is dried before removal from the electrode. In other embodiments, particularly when the web has sufficient wet strength, it can be stripped wet from the electrode and then dried.

Preferred fibers for use in the invention are fine denier 50 synthetic resin staples and flocks of lengths ranging from about 100 microns upwards to about two inches in length. Preferred fibers are staples of length from about  $\frac{1}{8}$  inch to about one inch and of denier in the range from about one to about 15 denier. Mixed fibers of varying denier or of 55 varying lengths within the defined ranges, or of both mixed denier and mixed lengths may be employed for varied fabric effects. The fibers may be flocks, staples, strands, filaments, etc. of any of several synthetic resin materials. Suitable synthetic fibers include polyesters such as poly 60 (ethylene terephthalate), poly(dimethylenecyclohexane terephthalate) and the like; viscose fibers such as rayon; polyamides such as the nylons; acrylic fibers such as polyacrylonitrile and modacrylic fibers and the like. Other fibers than the synthetic ones, such as mineral fibers and 65 cellulosic pulps may be employed in other embodiments of the invention. The selected fibers must be capable of being dispersed in the aqueous suspension, and should have a surface charge associated with each fiber.

Also dispersed in the aqueous suspension with the fibers 70 is a binder which also carries a charge so that it is also attracted to the electrode. Usually the binder is in suspension as in a colloidal dispersion or latex of resin particles

but in some embodiments the binder resin is carried on the surface of the fibers in the suspension. For anodic deposition, the fiber and binder will both be charged negative (anionic) and usually, but not in all instances, this charge is imparted by the action of an anionic surface active agent which is also in the aqueous medium. In other embodiments the suspended materials may be all charged positive for deposition at the cathode. In those embodiments, cationic resins and surfactants would be employed. In the following descriptions the more preferred anionic depositions are described in detail. However, the invention may be used for cationic deposition by using cationic resins and surfactants.

In those embodiments that employ dispersed resin particles separated from the fibers in the suspension, the selected resin is one that will coagulate or precipitate by being discharged at the anode, preferably being deposited as a wet gel or adhesive which provides a cohering binder for the wet deposit of fibers, and which becomes the dry fabric binder upon drying. Aqueous suspensions of resins suitable for deposit at the anode are latex suspensions of acrylic acid homopolymer or copolymers thereof with other acrylate or styrene monomers, of polyurethane resins or the like, of polyvinyl latex such as polyvinyl chloride, and a carboxy modified butadiene/acrylonitrile copolymers such as Hycar® 1572 and the like.

In those embodiments having the resin coated on the fibers in suspension, suitable resins for the purpose include resins for electrocoating paints in volatile, non-aqueous solvents such as Cyanamid XE-4010 Resin which is a solution of styrene-alkylacrylate-acrylic acid copolymer in a volatile nonaqueous solvent.

The concentration of both the fibers and the resin in the aqueous carrier are very important factors determining the consistency of the fabric that will be formed by electrophoretic deposition. To make a loosely matted, porous and permeable non-woven flocculent fabric according to the present invention, we employ aqueous dispersions having about one-fourth percent to about one percent by weight of the fine denier fibers in suspension and having about 0.05 to 0.2 percent by weight of resin solids in the suspension. It is important to keep the fiber suspension sufficiently dilute to avoid fiber entanglement and consequent coagulation of the fibers in suspension. Furthermore, and most important to the invention, it is necessary to work with the very dilute baths in order to obtain a desired high fiber to binder ratio in the fabric product. The fiber to resin ratio (by weight) in the aqueous electrolyte suspension is usually in the range from about two to about five parts by weight fiber to one part binder. Too little resin in relation to the amount of fibers will cause defective bonding of the fabric and too much will produce too dense a resin deposit. At higher concentrations of fiber in the suspension the fibers tend to tangle and coalesce, causing uneven deposits of fibers in the fabric.

The electrodeposition rates of the several sizes and kinds of fibers and of various resins in the aqueous suspension usually will vary, with the result that the relative proportions of the same elements in the fabric deposit will not usually correspond directly to their relative proportions in the aqueous suspension. Generally, it is found that in a suspension of mixed fiber lengths, shorter fibers tend to deposit at a faster rate than longer fibers of the same denier. Also, the fibers generally tend to deposit at rates slower than the deposition rates for the binder resins (except in those embodiments where the binder is bound to the fiber surface in the suspension). The result is that for a given composition of the suspension, the relative proportion of fiber to binder usually will be lower in the deposit than the proportion of fiber to binder in the suspension (with the exception already noted) and the same is usually true of the relative proportions of shorter and longer fibers when mixed fibers of several lengths are used.

Fabrics made in accordance with the present invention have much higher fiber to binder ratios than the fabric deposits described in the aforementioned Heron patent, and it was an object of the present invention to provide a process that could produce evenly deposited non-woven fabrics with fiber to binder ratios high enough to avoid the stiff, non-porous texture caused by higher resin concentration. It was found that such high fiber to binder ratios in the deposited fabric are obtained only by using dilute aqueous dispersions having not more than about one percent fiber and not more than about 0.2% resin in the electrolyte bath.

Most of the aqueous dispersions of resins that are commercially available have been provided with an anionic surfactant as an emulsifier or dispersing agent for dispersion of the resin solids in a latex. In some instances the presence of no more than this already provided amount of surfactant in the total suspension is found to be sufficient to act also as a dispersant and charge agent for the fibers. In most cases however, the presence of an additional amount of the same or another anionic surfactant will be needed to provide a surface charge for the fibers in suspension. When necessary, the fibers can be precoated with a concentrated surfactant to further assist fiber dispersion as the precoated fibers are stirred into the aqueous bath. In some instances the fibers are precoated with an insoluble resin binder which remains fixed on the fiber surface after the coated fibers are dispersed in the bath. A particularly suitable class of anionic dispersion agents for dispersing the fiber and binder in the bath are the high molecular weight polyacrylic acid having molecular weight ranging from about 5 to about 15 million. In addition to its dispersing function in the bath, this agent also behaves as a binder and thereby improves the wet and dry strength of the fabrics.

Effective concentration of the dispersion agent, when used, will be well below 0.1 percent of the total weight of the aqueous suspension and usually will be in the range from about .001 to .01 percent by weight.

In the cell, the working electrode surface may be any suitable electrically conducting material such as carbon, noble metals, other conductive metals that are electrochemically inactive or non-noble metals which are electrochemically active. The latter metals when used at the anode will be ionized in the aqueous medium to some extent during the electrodeposition and this may affect the deposition characteristics, particularly the coagulation of resins. Such anode metal ionization effect is not essential to the invention, but it may be present, and even may be advantageous in some cases. It is preferable to select an electrode with a smooth polished surface to facilitate removal of the fabric deposit from the electrode. Aluminum is found to be an anode that is quite suitable for the purpose in all respects and is most particularly advantageous because of its relative economy. Other suitable electrode materials include iron and steel and particularly stainless steel, as well as copper, zinc, cadmium, nickel and the like. The electrode for deposition may be shaped to the desired shape of the fabric product. For making fabric sheets, a plate or cylindrical rotating drum or a continuous metal belt may be employed as the electrode. For making continuous tubing, a cylinder electrode of suitable length may be provided, immersed in the aqueous bath with means for continuously drawing the formed fabric tube from one end of the cylinder. Individual articles such as cups, mitts, stocking shapes and the like can be formed on appropriately shaped individual electrodes. The counter electrode may be any suitable electrode material and in a preferred embodiment, the metal walls of the tank holding the electrolyte bath is the counter electrode.

The operating voltage is selected to be high enough for suitably rapid deposition, but not so high as to cause excessive electrolysis with consequent excessive gas for-

## 5

mation. Optimum voltage will usually be in the range from about 90 to about 200 volts and most often about 125-175 volts, varying within the range according to the selected electrodes and the composition of the bath. Some slight electrolysis at the working electrode is necessary in some embodiments to generate positive ions for reaction with the suspended particles near the electrode surface. For example, at the anode, hydrogen ion generated by electrolysis will diffuse outward into the deposits and discharge some of the attracted particles that have not reached actual contact with the electrode surface.

It is possible to vary the texture, thickness, strength, porosity, appearance, etc. of the web fabric products by varying the selection of fiber and resin materials and the selection of process conditions within the ranges already described. Generally, strength of the fabric is increased as fiber length is increased and as resin concentration is increased and as deposition voltage increases. Longer fibers tend to deposit less evenly than short fibers and the fabric of short fibers tends to be more densely packed and less porous than the fabrics of longer fibers. Increasing the proportion of resin to fiber will cause a stronger, denser and less porous product. Thickness of the deposit will depend mostly on the processing time, applied voltage and the concentrations of fibers and binder in the bath. Deposits from about 5 mils up to about one inch thick can be made in some instances, but for most uses fabric thicknesses of about 30 mils to about  $\frac{1}{8}$  inch thick will be preferred. We prefer to use fine denier fibers to obtain a soft, pliable fabric. Fibers heavier than about 15 denier will result in very coarse fabrics.

Natural fibers such as wood pulp, wool and some mineral fibers have fibrils which would act as tiny hooks to make the fibers self-bonding in a web, and in some instances hydrogen bonding can take place with further increased strength, but the synthetic filaments used in this invention do not have such self-bonding characteristics, so it is especially necessary to provide a well dispersed bonding resin within the fibrous web. Without a binder in the suspension, the synthetic fiber would gather at the electrode but would fall away when the electric current was stopped. The most even distribution of fiber and resin throughout the fabric is obtained by precoating the fibers with a resin binder that imparts a surface charge on each fiber. When separate resin latex particles and fibers are dispersed together, the resin deposited in the fabric will tend to be most concentrated at the fabric side nearest the electrode and the proportion of binder to fiber will tend to diminish outwardly through the fabric.

In some embodiments, particularly when mixed fiber lengths are used, it is found that the web product will vary in composition from a relatively smooth inner surface nearest the electrode where shorter fibers and more resin predominate, outwardly to a flocculent or even fleecy outer surface where the longer fibers are more dominant. This range of compositions across the fabric cross-section is in some instances an advantage because the inner, denser part of the web provides relatively more fabric strength while the outer surface has a more decorative and ornamental appearance.

## EXAMPLE I

Five grams of  $\frac{1}{8}$  inch long 3.0 denier polyester fiber, 2.5 grams of  $\frac{1}{4}$  inch 9.0 denier rayon and 1 gram  $\frac{3}{4}$  inch 3.0 denier rayon are soaked for 15 minutes in 250 ml. of a .01 wt. percent aqueous solution of Aerosol OT 75 (American Cyanamid Company) anionic surfactant. The fibers are removed from the solution, partially dried, then dispersed in 4500 ml. of a dilute aqueous latex which is prepared by mixing the following with water to make 4500 ml.:

3.5 ml. of a 45% solids latex of a copolymer of styrene and mixed lower alkyl acrylate and methacrylate esters (Accobond® 1094, American Cyanamid Company).

## 6

0.35 gram of hexamethoxymethylmelamine as a crosslinking agent for the styrene-acrylate copolymer.  
56.1 ml. of 10% solids aqueous emulsion of anionic polyurethane resin. (Cyanobond® U270, American Cyanamid Company).  
5 0.075 gram of polyacrylic acid (M.W.~15 million).

Final composition of the bath in wt. percent was:

|                              | Percent |
|------------------------------|---------|
| 10 Fiber                     | 0.185   |
| Cyanobond® U270 polyurethane | 0.12    |
| Accobond® 1094               | 0.03    |
| Hexamethoxymethylmelamine    | 0.001   |
| Polyacrylic acid             | 0.002   |
| 15 Remainder water.          |         |

The suspension was circulated from a reservoir through a 4 inch diameter, 5 inch deep stainless steel plating chamber by means of a Randolph pump. The plating chamber walls served as the cathode. The anode form on which the fabric was deposited was an aluminum cup  $1\frac{1}{16}$  inch in diameter and  $2\frac{1}{2}$  inch long. The cup was sprayed on its outer surfaces with Releasagen® H15-1 prior to immersing it in the bath. Upon application of 150 v. across the anode and cathode a deposit began to form. The voltage was applied for 4 minutes after which time the coated anode was removed from the bath, washed in water and dried at  $70^\circ$  C. for one-half hour. The deposit was removed from the form easily and had a dry weight of 1.17 grams and an average thickness of .030 inch. The product is a porous, non-woven fabric cup which is flexible as cloth but able to recover its original shape. It has a soft, fleecy outer surface and a somewhat smoother inner surface.

## EXAMPLE II

35 This embodiment employs fibers dispersed with the binder resin fixed to the surface of the fibers in the electro-coating bath.

35 Seventeen grams each of  $\frac{1}{8}$  inch long, 3.0 denier polyester fiber and  $\frac{1}{4}$  inch 9.0 denier rayon fiber are soaked in a 7.5 wt. percent solution in 2-ethoxyhexanol of XC4010 (American Cyanamid Company) acrylic resin. This resin is an acrylic copolymer having acrylic acid groups in the polymer chain. The fibers are removed from the resin solution, blotted dry and then vacuum dried at 45  $25^\circ$  C. overnight to remove the solvent. The resin-coated fibers are thoroughly beaten in 2 liters of water by a Waring Blender and then added to a plating tank containing 2.5 liters of water. Approximately 1 cc. of diethylamine is added to the bath to partially neutralize the carboxyl groups on the acrylic acid resin and thereby provide a good dispersion. Electrical conductivity of the bath is  $7.4 \times 10^{-5}$  ohm $^{-1}$  cm. $^{-1}$ .

45 The anode form and plating chamber are the same as described in Example I. Upon application of 150 v. for 55 two minutes, electrophoretic deposition of the fibers forms a fabric cup on the anode, which is stripped from the electrode, washed in water and dried at  $70^\circ$  C. for one-half hour. Dry weight of the fabric cup is 0.43 gram and the fabric walls are 0.010 inch thick.

## EXAMPLE III

55 A bath was prepared using the same materials and procedure, but only half the binder concentration described in Example I. Composition of the fresh bath before electro-deposition was:

|                           | Percent |
|---------------------------|---------|
| Fiber                     | .18     |
| Cyanobond® U270           | .06     |
| Accobond® 1094            | .02     |
| Hexamethoxymethylmelamine | .0005   |
| Polyacrylic acid          | .002    |

75 A deposit was formed at 150 v. for 4 minutes onto an aluminum anode cup  $1\frac{1}{16}$  inch in diameter and  $2\frac{1}{2}$  inch long. The dry deposit weighed 1.85 grams and had an

average thickness of 0.050 inch. The deposit was softer but had less strength than that produced in Example I due to the decreased binder content.

#### EXAMPLE IV

A bath was prepared using the same materials and procedure described in Example I but having only 30% of the binder concentration described in Example I. The bath composition was:

|                           | Percent |
|---------------------------|---------|
| Fiber                     | .18     |
| Cyanobond® U270           | .036    |
| Accobond® 1094            | .0012   |
| Hexamethoxymethylmelamine | .003    |
| Polyacrylic acid          | .002    |

Upon application of 150 v. across the cell for 4 minutes a deposit formed on the surfaces of the aluminum anode cup. The deposit had very low wet strength due to the low binder concentration.

#### EXAMPLE V

A bath was prepared using the same materials and procedure but about twice the total fiber concentration as in Example I. The final bath composition was:

|                           | Percent |
|---------------------------|---------|
| Fiber                     | .37     |
| Cyanobond® U270           | .12     |
| Accobond® 1094            | .04     |
| Hexamethoxymethylmelamine | .001    |
| Polyacrylic acid          | .002    |
| Remainder water           |         |

A deposit was formed at 150 v. for 2 minutes on an aluminum cup  $1\frac{1}{16}$  inch in diameter and  $2\frac{1}{2}$  inch long. The deposit had an average thickness of .030 inch.

#### EXAMPLE VI

This example is presented for comparison to illustrate certain advantages of the invention. A more concentrated bath was prepared by adding 12.2 g.  $\frac{1}{4}$  inch 9.0 denier rayon and 52.2 g. rayon floc to 2375 ml. of an aqueous latex to make a final bath composition of:

|                           | Percent |
|---------------------------|---------|
| Fiber                     | 2.6     |
| Cyanobond® U270           | 0.51    |
| Accobond® 1094            | 0.45    |
| Hexamethoxymethylmelamine | .015    |
| Remainder water           |         |

A deposit was formed on a 3 inch x 3 inch aluminum anode plate at 100 v. for 2 minutes. Dry weight of the deposited sheet removed from the electrode was 4.64 grams. The sheet had very uneven surface texture and was very stiff with more of the character of the polymeric binder than of the fibers.

#### EXAMPLE VII

In this example, the process produces a non-woven fabric having a gradation of polymer to fiber ratios across the thickness of the fabric with substantially more polymeric binder deposited at the inner side nearer the electrode than on the outer side of the fabric.

A bath is prepared by the procedure described in Example I, but containing 12 grams rayon flock, 5.9 grams of  $\frac{1}{8}$  ", 3.0 denier polyester fiber, 4.4 grams of  $\frac{1}{4}$  ", 3.0 denier rayon fiber and 140 ml. of a 10% solids latex Cyanobond® 4270 in 10 liters of deionized water. The composition of the bath in wt. percentage is:

|                 | Percent |
|-----------------|---------|
| Fiber           | 0.22    |
| Cyanobond® 4270 | 0.14    |
| Remainder water |         |

The deposit is formed by electrodeposition in the same

manner described in Example I. The fabric is deposited on the positive electrode, a  $2\frac{1}{2}$  " diameter, 5" long aluminum cylinder which has been sprayed with Releasagen® H15-1. The electrodeposition is carried out using 200 volts constant voltage for 3 minutes. The electrode is removed from the bath and the deposit is washed in deionized water while still on the cylinder. It is then carefully removed wet from the cylinder and drum dried for 4 minutes at  $120^{\circ}$  C. The fabric, which is about 30 mils thick, is soft and flexible and has a gradation of polymer to fiber ratio through the thickness of the fabric with the electrode side having relatively more polymer than the fleecy outer surface. This gradation of polymer to fiber ratio is visibly apparent by no more than visual observation of the two sides. The electrode side is smoother and stronger than the fleecy outer side. A photomicrograph of a cross section of the fabric shows the gradation of polymer concentration across the thickness of the fabric. The average composition of the entire fabric is measured and found to be 42% Cyanobond® 4270 and 58% fiber. The fleecy outer side of a 1.29 g. sample of the deposit is abraded to remove material from the fiber-rich outer surface. This material is analyzed and found to contain practically all fibers with no appreciable amount of polymer. Material abraded from the polymer rich side, the side deposited nearer the electrode, was analyzed and found to contain 54% Cyanobond® 4270 and 46% fiber, which is higher than the average polymer concentration. These tests and observations demonstrate the gradation of polymer concentrations across the thickness of the web, from a concentration well above average on the inner side to nearly all fibers at the outer surface. Also the micrographs clearly show gradual deposition of higher proportions of the longer fibers outward from the electrode side.

The foregoing examples illustrate several embodiments of the invention. These and various other embodiments of the invention have produced fabrics having tensile strengths (dry) from about 2 to about 19 pounds per inch. Variations and modifications of the invention which are not specifically described may be made within the scope of the invention as it is described herein and defined by the following claims.

We claim:

1. A process of making non-woven fabric articles comprising depositing fibers and resin by application of a suitable voltage at an electrode surface from an aqueous bath in which such fibers and resin are dispersed and removing the fabric deposit from said electrode, the fiber in said bath being present at concentration less than one wt. percent and the resin in said bath being present at concentration less than 0.2 wt. percent, said percentages based on the total weight of the aqueous bath, and the wt./wt. ratio of fiber to resin being in the range from one to five parts fiber to one part resin in said bath.
2. A process defined by claim 1 wherein said fibers are of length in the range from about 100 microns to about two inches and of denier in the range from about 1 to about 15 denier.
3. A process defined by claim 2 wherein said fibers are synthetic resin fibers.
4. A process defined by claim 1 wherein said fiber and resin are dispersed with the resin fixed to the surface of said fibers in the dispersion.
5. A process defined by claim 1 wherein the ratio of fiber to binder obtained in the fabric deposit is in the range from about one to about five parts by weight fiber to one part resin in the fabric deposit.
6. A fabric made by the process defined in claim 1, having a gradation of polymer to fiber ratios across the fabric cross section.
7. A fabric made by the process defined by claim 1 having dry tensile strength in the range from about 2 to about 19 pounds per inch.

8. A fabric made by the process defined by claim 1 having thickness in the range from about 30 to about 125 mils.

## References Cited

## OTHER REFERENCES

- |           |         |                  |           |
|-----------|---------|------------------|-----------|
| 2,858,256 | 10/1958 | Fahnoe           | 204—4     |
| 3,061,525 | 10/1962 | Grazen           | 204—16    |
| 3,449,230 | 6/1969  | Heron et al.     | 204—180 R |
| 3,449,227 | 6/1969  | Heron et al.     | 204—180 R |
| 3,556,969 | 1/1971  | Mizuguchi et al. | 204—180 R |
| 3,626,041 | 12/1971 | Fields           | 204—180 R |

## FOREIGN PATENTS

- |           |        |               |        |
|-----------|--------|---------------|--------|
| 953,506   | 7/1962 | Great Britain | 204—16 |
| 1,070,343 | 6/1967 | Great Britain | 204—16 |

5 JOHN H. MACK, Primary Examiner

T. TUFARIELLO, Assistant Examiner

U.S. Cl. X.R.

10 204—4, 181